

Patented Aug. 30, 1927.

1,640,706

## UNITED STATES PATENT OFFICE.

MORRIS CHARLES LAMB, OF BIRMINGHAM, LONDON, ENGLAND, ASSIGNEE TO ROHM & HAAS COMPANY, INC., OF PHILADELPHIA, PENNSYLVANIA.

### TREATING OF LEATHER.

No Drawing. Original application filed June 9, 1925, Serial No. 33,052, and in Great Britain April 27, 1925. Divided and this application filed March 6, 1926. Serial No. 32,840.

This invention relates to the treatment of leather and more particularly tanned leather which has already been dyed and represents a division of application No. 36,052 filed June 9, 1925, the object of the invention is the lubricating of the fibres of the leather in order to improve its quality.

According to this invention I treat the leather with an emulsion of a compound containing a naphthalene nucleus in association with an oil or fat of a type suitable for lubricating the fibres of the leather in accordance with known practice. The oil may be of animal, vegetable, or mineral nature. The leather employed may be tanned either by vegetable or mineral tanning agents or dressed by the oil or aldehyde process, the treatment by the compound containing the naphthalene nucleus, more particularly hydrogenated naphthalene, effecting an equal distribution and solubilization of the oil and fatty matter throughout the leather. The hydrogenated naphthalene may be used in a soluble or finely divisible form or in an emulsified form obtained by the employment of emulsifying agents such as sodium, potassium or ammonium ricinoleate, hydrogenated phenol or resol soaps, sulphonated or soluble oils of vegetable, animal, or mineral origin, the salts of sulphonated aromatic acids, or aromatic acids used either alone or in conjunction with each other. The term "emulsion" as used in this specification is intended to cover an ordinary emulsion or a solution, where this is feasible, of the naphthalene compound.

The naphthalene compound can also be used in conjunction with halogen, or other hydrocarbon compounds.

The following is an example of the treatment of a leather in accordance with this invention, the example including the previous dyeing method:—

Vegetable, mineral tanned, or oil dressed or aldehyde leather is first wetted out by any of the ordinary methods, by drumming, paddling or steeping in water at any convenient temperature, and is then subsequently dyed with coal-tar or natural dyestuff. The leather after dyeing is then subjected to a special treatment with 3 per cent to 6 per cent of an emulsion of any suitable oil for the purpose of lubricating the fibres of the leather, the emulsion being used in conjunction with an emulsion or compound of naphthalene, either with or without the addition of tri-chlorethylene, tri-chlorethane, or other hydrocarbon compound.

What I claim and desire to secure by Letters Patent of the United States is:—

1. A process for treating leather for the purpose of lubricating its fibres, which consists in treating the leather with a non-acid emulsion of hydrogenated naphthalene in association with an oily substance.

2. A process of treating tanned leather subsequently to dyeing, which consists in treating the leather with a non-acid emulsion of hydrogenated naphthalene in association with an oily substance for lubricating the fibres of the dyed leather.

MORRIS CHARLES LAMB.